

# UNITED STATES PATENT OFFICE.

JAMES F. O'BRIEN, OF CHICAGO, ILLINOIS.

## EXPLOSIVE.

1,132,873.

Specification of Letters Patent. Patented Mar. 23, 1915.

No Drawing.

Application filed October 14, 1913. Serial No. 795,060.

To all whom it may concern:

Be it known that I, JAMES F. O'BRIEN, a citizen of the United States, residing at Chicago, in the county of Cook, State of Illinois, have invented new and useful Improvements in Explosives, of which the following is a specification.

This invention relates to an explosive whose characteristic ingredients are ammonium perchlorate and a liquid nitrated coal

tar product, preferably liquid binitrotoluene; with carbon, comminuted wood, or equivalent, and with or without a nitrate of an alkali metal, preferably sodium nitrate.

It may be stated as the broad object of the present invention to provide an easily manufactured ammonium perchlorate explosive of high efficiency in a water proof, plastic form.

There are many other objects and corresponding advantages of my present explosive; but all other objects and advantages of my present explosive may be grouped under the above prime objects.

One object is to use materials which may be easily and freely obtained on the market or which may be manufactured from easily obtainable substances; enabling me to manufacture in large quantities from materials obtainable in the United States.

As to efficiency, it is explained in the specification hereinafter how my new explosive has not only a great gas volume without an unduly high temperature but also has a very high speed of action; so that, although the explosion temperature may be lower than that of dynamite, gelatin or other explosives which may be compared with my present explosive, the effective work performed by my present explosive is much greater than the work performed by an equal weight of the best commonly known and used explosives; and in the comparison of my explosive with other explosives on the cost for cost basis, my explosive far exceeds the others in point of effectiveness for a given expenditure.

The feature of low temperature is one of great moment; and it is caused in no small degree in my explosive by the formation of sodium chlorid during combustion. The sodium chlorid absorbs a great quantity of heat, thereby greatly reducing the temperature, and renders my explosive especially suited for work in coal mines and the like

where an explosive is required to do effective work at low temperature.

The inclusion of binitrotoluene in my composition has mainly two effects; first, to make the explosive plastic and water-proof and, second, to accelerate the speed of detonation so that the effectiveness of the explosive for blasting of all sorts is greatly increased. Speed is also induced by the carbon.

Ammonium perchlorate has many advantages for explosive use; it is commercially available on the market or by manufacture and it is safe to handle. Its safety is caused by the comparatively high temperature required for its decomposition; but this requirement is also the cause of slow detonation of the ammonium perchlorate explosives heretofore proposed.

Ammonium perchlorate explosives generally show a high temperature and great gas volume, but they are generally lacking in the third prime requisite of explosive efficiency—high speed of reaction. In my explosive I increase the

speed of action by the use of a liquid nitrated coal tar product (preferably the so-called the liquid binitrotoluene) and then cause further increase of speed by using free carbon, in the composition. The binitrotoluene in liquid form seems to bring the active

ingredients into more intimate contact than can be the case with solid ingredients exclusively; while the office of the free carbon is to cause initial breaking down of the perchlorate into chlorate. The maximum amount of carbon needed is that sufficient to cause the reaction; being about 5.5% of the amount of perchlorate; although much smaller amounts give notable results. The carbon I prefer to supply in the form of finely divided charcoal, or I may provide it by partially roasting sawdust so that its surface is more or less carbonized.

I prefer to make my explosive in varying grades, varying from a grade of greatest effective strength to a grade of lowest effective strength. In my explosive of greatest power I prefer to use only ammonium perchlorate, liquid binitrotoluene, carbon and comminuted wood in the form of saw dust. In my next highest grade I prefer to use a certain amount of a nitrate, preferably sodium nitrate; and in the succeeding grades the amount of sodium nitrate is increased and that of ammonium perchlorate decreased

until, in the lowest grade, the maximum amount of sodium nitrate is used. I may use potassium, calcium or barium nitrate or ammonium nitrate; but sodium nitrate is generally to be preferred on account of its cheapness and availability in large quantities on the market.

The following table gives my preferred forms and indicates the range over which the composition may vary.

|    | NH <sub>4</sub> ClO <sub>4</sub> | NaNO <sub>3</sub>  | Liquid binitrotoluene.         | Sawdust.                      | C.                                                                                |
|----|----------------------------------|--------------------|--------------------------------|-------------------------------|-----------------------------------------------------------------------------------|
| 15 | No. 0.....                       | 65                 | .....                          | 15                            | 20 3.5                                                                            |
|    | No. 1.....                       | 44                 | 32                             | 10                            | 14 2.4                                                                            |
|    | No. 1 <sup>a</sup> .....         | 36.5               | 26.5                           | 15                            | 22 2.0                                                                            |
|    | No. 2.....                       | 32                 | 43                             | 10                            | 15 1.75                                                                           |
|    | No. 2 <sup>a</sup> .....         | 28                 | 34                             | 15                            | 23 1.5                                                                            |
|    | No. 3.....                       | 20                 | 55                             | 10                            | 15 1.1                                                                            |
|    | No. 3 <sup>a</sup> .....         | 20                 | 42                             | 15                            | 23 1.1                                                                            |
| 20 |                                  |                    |                                |                               |                                                                                   |
|    | Gases.                           | Calories per kilo. | Maximum explosion temperature. | Liters expanded gas per kilo. | Gaseous products of explosion.                                                    |
| 25 |                                  |                    |                                |                               |                                                                                   |
|    | Liters per kilo.                 |                    | Degrees C.                     |                               |                                                                                   |
|    | No. 0.....                       | 877                | 825                            | 2,240                         | 8,060 (H <sub>2</sub> O, HCl, N, CO <sub>2</sub> , Small amount CO <sub>2</sub> ) |
|    | No. 1.....                       | 612                | 1,149                          | 2,611                         | 6,457 (H <sub>2</sub> O, CO <sub>2</sub> , N, Trace CO)                           |
| 30 | No. 1 <sup>a</sup> .....         | 763                | 782                            | 2,113                         | 6,661 (H <sub>2</sub> O, CO, N, Small amount CO <sub>2</sub> )                    |
|    | No. 2.....                       | 556                | 1,103                          | 2,585                         | 5,816 (H <sub>2</sub> O, CO <sub>2</sub> , N, Small amount CO)                    |
|    | No. 2 <sup>a</sup> .....         | 731                | 739                            | 2,053                         | 6,221 (H <sub>2</sub> O, CO, N, Small amount CO <sub>2</sub> )                    |
|    | No. 3.....                       | 495                | 1,048                          | 2,564                         | 5,138 (H <sub>2</sub> O, CO <sub>2</sub> , N, Small amount O)                     |
| 35 | No. 3 <sup>a</sup> .....         | 685                | 715                            | 2,022                         | 5,754 (H <sub>2</sub> O, CO, N, Small amount O)                                   |

In this table I give the maximum quantities of carbon needed; smaller amounts may be used. The carbon may be in the form of finely divided charcoal; or it may be supplied by partially carbonizing the sawdust or equivalent material used.

The No. 0 explosive is seen to have the greatest absolute expansion; and it also has the greatest speed of action. It is designed to be primarily useful in open blasting work; its detonation resembles very much that of nitro-glycerin. It leaves gaseous products including carbon monoxid and hydro-chloric acid, and for this reason is unsuited to inclosed work, as in mines, etc. Explosive No. 0 is of extremely great strength. Its expanded volume in proportion to its initial weight is greater than that of 55% gelatin dynamite; and its rate of detonation is so high that its efficient work is greater and better than that of 75% gelatin dynamite.

Explosive No. 1 contains 32% of sodium nitrate; and its formula is so arranged that there is little or no carbon-monoxid in its resultant gaseous products; the carbon being taken up in carbon dioxid. There is no hydro-chloric acid, the chlorin being deposited in a sodium chlorid deposit amounting

to some considerable percentage of the original weight of the explosive. No. 1 is the strongest and most effective explosive adapted for interior work, producing no noxious or poisonous gases and depositing sodium chlorid which has the effect of greatly reducing the temperature and absorbing the heat of the explosion. This explosive is of the "non-flame" type.

Explosives Nos. 2 and 3 are similar to No. 1 excepting that the amounts of ammonium perchlorate are progressively less and the amounts of sodium nitrate are progressively greater than in No. 1. In each of the explosives Nos. 2 and 3 the composition is made so that the products of combustion are practically the same as in explosive No. 1 except that, in addition, explosives Nos. 2 and 3 also deposit some sodium carbonate. Explosives Nos. 1, 2 and 3 are thus particularly adapted to interior or confined work while explosive No. 0 is particularly adapted to open work.

In order to provide explosives with rates of detonation corresponding to those of Nos. 1, 2 and 3 and with corresponding, or nearly corresponding strength, I have provided explosives 1<sup>a</sup>, 2<sup>a</sup>, 3<sup>a</sup>. These explosives 1<sup>a</sup>, 2<sup>a</sup> and 3<sup>a</sup> differ from the respective explosives Nos. 1, 2 and 3 only in slight changes of proportions of ingredients; the proportions in explosives 1<sup>a</sup>, 2<sup>a</sup> and 3<sup>a</sup> being such that the gaseous products contain carbon monoxid instead of carbon dioxid. The net results of having carbon monoxid in the resultant gaseous products is to greatly increase the volume of the heated expanded gases. For instance, No. 1<sup>a</sup> is slightly cheaper to manufacture than No. 1 while its expanded volume is greater than the expanded volume of No. 1.

I provide a series of explosives of graduated strengths suitable both for interior and exterior work. The explosives having carbon dioxid in their gaseous products are to be preferred for general all around work. For work in the open, exclusively, explosives Nos. 1<sup>a</sup>, 2<sup>a</sup> and 3<sup>a</sup> and explosive No. 0 are to be preferred on account of greater effectiveness of work performed for a given cost.

With regard to all of the above described explosives I desire to emphasize first the qualities which the liquid binitrotoluene imports into the composition. The liquid binitrotoluene not only makes the explosive plastic and water-proof, but adds a great many other desirable physical qualities, chief among which is the adaptability of the powder to cartridge formation. I would also emphasize the ease with which my explosive is formed. The liquid binitrotoluene is simply mixed with the other ingredients until it thoroughly coats and surrounds all of them. The explosive is then ready for packing into cartridges for shipment and

use. Speed of action is also induced by the liquid binitrotoluene; and the addition of the free carbon further increases the speed to the maximum. The great efficiency of my present explosive depends upon its great speed of action. With high detonation speed my explosives have great effective strength without a high temperature of combustion. The speed of action, of course, varies with the different compositions, being greatest in No. 0 and least in Nos. 3 and 3<sup>a</sup>. No. 0 has a speed of action resembling that of nitro-glycerin while Nos. 3 and 3<sup>a</sup> have a speed of action more like ordinary black powder, having, however, a much greater strength than that of black powder. No. 3 has an effective strength equal to that of about 30% dynamite, No. 2 to 40% dynamite and No. 1 to 65% dynamite; while the respective rates of detonation are approximately those of dynamites.

With regard to all of the above described explosives it may be particularly stated that they are non-deteriorating under ordinary atmospheric conditions or when exposed to moisture; they will not decompose or change in any manner through long periods of time. None of them can be detonated by mere concussion, friction, jar or vibration; requiring both concussion and heat for detonation, whether confined or unconfined. When supplied with both concussion and heat, as from a cap, they each and all detonate perfectly whether confined or unconfined. They may each be shot into without detonation. When ignited in the open, without concussion, explosive No. 0 flashes nearly as quickly as

black powder, explosive No. 1 burns at a rather lively rate, explosive No. 2 at a slower rate while explosive No. 3 is ignitable but will not continue to burn unless the combustion is forced. These properties make my explosives exceedingly safe to handle and at the same time give positive and reliable results when detonated in the correct manner. My explosive has all of the desirable features of the various nitro-glycerin products without any of their objectionable features; it has their strength and effectiveness but none of their dangers.

I claim—

1. An explosive, comprising ammonium perchlorate not less than twenty parts of weight, sodium nitrate not more than fifty-five parts by weight, liquid binitrotoluene ten to fifteen parts by weight, saw dust fourteen to twenty-three parts by weight, and free carbon about five per cent. of the weight of the ammonium perchlorate.

2. An explosive, comprising ammonium perchlorate twenty to sixty-five parts by weight, sodium-nitrate not more than fifty-five parts by weight, liquid binitrotoluene ten to fifteen parts by weight, sawdust fourteen to twenty-three parts by weight, and free carbon one to three and one-half parts by weight.

In witness that I claim the foregoing I have hereunto subscribed my name this eighth day of October, 1913.

JAMES F. O'BRIEN.

Witnesses:

M. ROBBINS,  
JAMES T. BARKELEW.

Copies of this patent may be obtained for five cents each, by addressing the "Commissioner of Patents, Washington, D. C."